

2,847,388

FOUNDRY SAND CORE COMPOSITIONS AND  
METHOD OF PREPARATION

Stuart H. Rider, Longmeadow, Thomas Anas, Springfield, and William D. Burke, West Springfield, Mass., assignors to Monsanto Chemical Company, St. Louis, Mo., a corporation of Delaware

No Drawing. Application April 5, 1954  
Serial No. 421,194

10 Claims. (Cl. 260—17.3)

This invention relates to foundry sand core compositions. More particularly, this invention relates to foundry sand core compositions comprising a mixture of a suitable core sand with a modified core oil binder.

It is conventional practice to prepare metal castings in molds having hardened sand core compositions positioned therein to define internal openings in the casting. Such sand cores are prepared by shaping a mixture of sand and a suitable core binder in any suitable mold such as a core box, removing the shaped mixture from the mold and hardening the same by baking. Satisfactory core binders should not interfere with the workability of the sand and should impart satisfactory green strength and bake strength to cores molded from the mixture of sand and binder. Each of these factors are of importance in that, for example, the mixture of sand and binder is shaped in the core box only with difficulty if it is sticky (i. e., has poor workability), this being particularly true if the core is to be shaped by a "blowing" process wherein the mixture of sand and binder is blown into and compacted in a core box by air pressure. Similarly, green strength and bake strength are important since the shaped core should not be readily deformable prior to or during baking and metal casting operations.

One widely used type of core binder is a drying oil-containing binder (commonly referred to as a core oil) which is normally compounded with the core sand in conjunction with other additives, including cereals such as flour, restricted amounts of water, etc. Although core oil-containing binder compositions, generally speaking, do not impair the workability of the sand and impart satisfactory green strength and bake strength to cores molded from the mixtures of sand and binder, the use of core oils is still attendant with various disadvantages.

A major disadvantage encountered in the use of core oil-binder compositions is the relatively long baking cycle that is required to develop satisfactory bake strength in the core. Although various proposals have been advanced in an effort to solve this problem, such proposals have generally proved to be unsatisfactory in one respect or another. This problem is particularly accentuated since it is desirable to reduce baking time without materially affecting other variables such as the workability of the sand-binder mixture and the green strength of the cores molded therefrom.

Accordingly, an object of the present invention is the provision of foundry sand core compositions which will develop satisfactory bake strength after a comparatively short baking cycle.

Another object is the provision of foundry sand core compositions comprising a mixture of a core sand with a modified core oil-binder composition.

A further object is the provision of a process for the preparation of foundry sand cores.

These and other objects are attained by replacing from 20 to 50% by weight of the core oil in a core oil-binder composition with a corresponding amount by weight of a tetra-, penta- or hexamethylol melamine fully etherified

with a saturated aliphatic monohydric alcohol having from 1 to 6 carbon atoms, shaping the mixture to form a core and baking the core for from 30 to 45 minutes at a temperature of about 350 to 450° F.

5 The following examples are given in illustration and are not intended as limitations on the scope of this invention. Where parts are mentioned, they are parts by weight.

## EXAMPLE I

10 Prepare two foundry core mixes, the compositions of which are set forth in Table I, and mold a plurality of briquettes from each of the compositions in a suitable core box. In molding the briquettes, it is found that both 15 of the mixes have good workability and that the briquettes molded therefrom have satisfactory green strength. The green briquettes are readily stripped from the core box without the use of mold release agents or lubricants. Bake the briquettes prepared from the two mixes in a 20 suitable oven at a temperature of about 400° F., one portion of the briquettes of each mix being baked for 30 minutes and the other portion of each mix being baked for 60 minutes. Test the baked briquettes for tensile strength in accordance with the American Foundrymen's 25 Society test for tensile strength (Foundry Sand Handbook, pages 86-95, 6th edition, 1952, American Foundrymen's Society, Chicago, Illinois). The results of the test are set forth in Table II.

Table I.—Core mixes

| Mix    | Ottawa Sand (parts) | Corn Flour (parts) | Water (parts) | Raw Linseed Oil (parts) | Butylated Hexamethylol Melamine (parts) |
|--------|---------------------|--------------------|---------------|-------------------------|-----------------------------------------|
| 1----- | 1,000               | 10                 | 35            | 10                      | 0                                       |
| 2----- | 1,000               | 10                 | 35            | 5                       | 5                                       |

Table II.—Average tensile strength of baked briquettes

| Mix    | Tensile Strength, p. s. i.  |                             |
|--------|-----------------------------|-----------------------------|
|        | Briquettes Baked 30 Minutes | Briquettes Baked 60 Minutes |
| 1----- | 110                         | 189                         |
| 2----- | 190                         | 261                         |

50 With reference to Table II, it is seen that the briquettes prepared from the core oil-binder composition modified with butylated hexamethylol melamine developed a satisfactory bake strength after 30 minutes of baking whereas the unmodified composition required 60 minutes of baking in order to obtain satisfactory bake strength. In 55 other words, a 50% reduction in baking time was realized.

When Example I is repeated using either butylated tetra-methylol melamine or butylated pentamethylol melamine in place of butylated hexamethylol melamine, it found 60 that the resultant compositions have satisfactory workability and that briquettes molded therefrom have satisfactory green strength and bake strength. It is also found that, as in the case of Example I, a satisfactory bake strength is obtained after about 30 minutes of baking at 400° F.

## EXAMPLE II

As a further illustration of the present invention, prepare a plurality of foundry sand core mixes having the compositions set forth in Table III. Mold briquettes 70 from the compositions and bake and test the same in accordance with the procedure set forth in Example I. The results are set forth in Table IV.

When preparing the briquettes, it is noted that there is no significant difference in workability from mix to mix and it is also noted that all of the molded briquettes have satisfactory green strength.

Table III.—Core mixes

| Mix    | #60 Ottawa Sand (parts) | Corn Flour (parts) | Water (parts) | Core Oil <sup>1</sup> (parts) | Ether (parts)                          |
|--------|-------------------------|--------------------|---------------|-------------------------------|----------------------------------------|
| 1..... | 1,000                   | 10                 | 35            | 10                            |                                        |
| 2..... | 1,000                   | 10                 | 35            | 7.5                           | Methylated Hexamethylol melamine, 2.5. |
| 3..... | 1,000                   | 10                 | 35            | 7.5                           | Butylated Hexamethylol melamine, 2.5.  |

<sup>1</sup> A typical commercial core oil comprising linseed oil modified with slower drying oils.

Table IV.—Average tensile strength of baked briquettes

| Mix    | Tensile Strength, p. s. i.  |                             |
|--------|-----------------------------|-----------------------------|
|        | Briquettes Baked 30 Minutes | Briquettes Baked 60 Minutes |
| 1..... | 150                         | 345                         |
| 2..... | 318                         | 319                         |
| 3..... | 334                         | 342                         |

As the results of the foregoing tests illustrate, a 50% reduction in baking time is realized with Mixes 2 and 3 prepared in accordance with the present invention as compared with Mix No. 1 prepared from an unmodified core oil-binder composition.

Equally satisfactory results are obtained when mixes are prepared by blending 100 parts of #60 Ottawa sand, 10 parts by weight of corn flour and 35 parts by weight of water with a mixture of 7.5 parts by weight of the commercial core oil and 2.5 parts by weight of methylated or hexylated tetramethylol melamine. It is found that such mixes have good workability and that briquettes molded therefrom have satisfactory green strength. When such briquettes are baked for 30 minutes at a temperature of about 400° F. and then tested for tensile strength in accordance with the procedure set forth in Example I, it is found that there is no significant difference in bake strength as compared with the briquettes of Mixes 2 and 3 of Example II which are similarly baked for 30 minutes.

The etherified methylol melamines to be used alone or in admixture with one another in accordance with the present invention are the tetra-, penta- and hexamethylol melamines fully etherified with saturated aliphatic monohydric alcohols having from 1 to 6 carbon atoms. The etherified compounds are easily prepared by reacting tetra-, penta- or hexamethylol melamine with a large excess of an aliphatic saturated monohydric alcohol having from 1 to 6 carbon atoms, such reaction being conducted under strongly acid conditions at a temperature of about 10-40° C. If desired, mixed ethers may be prepared by an interchange reaction wherein an aliphatic alcohol having 2 or more carbon atoms is added to a methylol melamine etherified with an aliphatic alcohol having a lesser number of carbon atoms while the etherified melamine is in solution in an aliphatic alcohol which also has a lesser number of carbon atoms. Thus, when butanol is added to a solution of methylated hexamethylol melamine in methanol, the butanol reacts with the methylated melamine compound, replacing the methyl groups with butyl groups. The number of groups to be replaced in this fashion is dependent on the molar ratios of the reactants so that one, several or all of the aliphatic groups originally present may be replaced by higher aliphatic groups. Representative etherified methyl melamines of the present invention include the methylated, ethylated, propylated, butylated, pentylated and

hexylated tetra-methylol melamines, pentamethylol melamines and hexamethylol melamines. As indicated, mixed ethers of tetra-, penta- or hexamethylol melamines containing, for example, both methyl and butyl radicals or both methyl and hexyl radicals may also be used. Such etherified methylol melamines are liquid compounds of varying viscosity which are compatible with conventionally used core oils.

In accordance with the present invention, such etherified methylol melamines are used to replace a part of the core oil normally used in foundry sand core compositions. Numerous examples of core oils are known to those skilled in the art. Such core oils normally contain, as a base, a drying oil such as perilla oil, linseed oil, menhaden oil, the highly unsaturated polymers derived from cracked gasoline, etc.

When from about 20 to 50% by weight of such a core oil is replaced by an equal amount by weight of one or more of the etherified methylol melamines of the present invention and the mixture is compounded with a suitable core sand and the other conventional ingredients in the manner known to those skilled in the art, there is obtained a fast baking composition having properties otherwise equivalent to the properties of unmodified core oil-binder compositions.

Any sand suitable for use with commercial core oils may be used to prepare the cores, such as geauga float sand, New Jersey silica sand, Ottawa foundry sand, Ottawa silica sand, Portage crude sand, Ohio geauga sand, Providence core sand, Wisconsin silko bank sand, etc. Such sands are preferably washed free from organic impurities prior to use.

For practical purposes, it is necessary to use a minor amount of water and a cereal such as corn flour, dextrin, wheat flour, oat meal, etc. in order that molded cores may have satisfactory green strength.

Generally speaking, satisfactory foundry sand core compositions of the present invention will comprise about 1000 parts of a suitable sand, about 7-20 parts of a mixture of about 50-80% by weight of a core oil with, correspondingly, about 50-20% by weight of an etherified methylol melamine of the present invention, about 7-15 parts of a suitable cereal and about 35 parts of water. Such compositions have good workability, being of particular utility in the preparation of "blown" cores. Cores molded from such compositions have satisfactory green strength and develop satisfactory bake strength within 30-45 minutes when baked at temperatures of 350-450° F. In general, a reduction in baking time of about 50% is obtained with the compositions of the present invention as compared with equivalent core oil-containing compositions free from etherified methylol melamines.

What is claimed is:

1. A foundry sand core composition consisting essentially of about 1000 parts by weight of sand, about 7-15 parts by weight of cereal, about 35 parts by weight of water and about 7-20 parts by weight of a mixture of about 50-80% by weight of a core oil with, correspondingly, about 50-20% by weight of a compound taken from the group consisting of tetra-, penta- and hexamethylol melamines fully etherified with saturated aliphatic monohydric alcohols having from 1 to 6 carbon atoms.
2. A foundry sand core composition as in claim 1 wherein the compound is a fully etherified tetramethylol melamine.
3. A foundry sand core composition as in claim 1 wherein the compound is a fully etherified pentamethylol melamine.
4. A foundry sand core composition as in claim 1 wherein the compound is a fully etherified hexamethylol melamine.
5. A foundry sand core composition as in claim 2 wherein the etherified tetramethylol melamine is methylated tetramethylol melamine.

6. A foundry sand core composition as in claim 2 wherein the etherified tetramethylol melamine is butylated tetramethylol melamine.

7. A foundry sand core composition as in claim 3 wherein the etherified pentamethylol melamine is butylated pentamethylol melamine. 5

8. A foundry sand core composition as in claim 4 wherein the etherified hexamethylol melamine is methylated hexamethylol melamine.

9. A foundry sand core composition as in claim 4 10 wherein the etherified hexamethylol melamine is butylated hexamethylol melamine.

10. A process for preparing a foundry sand core which comprises thoroughly intermingling about 1000 parts by weight of sand with about 7-15 parts by weight of cereal, about 35 parts by weight of water and about 7-20 parts by weight of a mixture of 50-80% by weight of a core oil with, correspondingly, about 50-20% by weight of a 15

compound taken from the group consisting of tetra-, penta- and hexamethylol melamines fully etherified with saturated aliphatic monohydric alcohols having from 1 to 6 carbon atoms, molding a core from said mixture and baking said molded core at a temperature of about 350-450° F. for about 30-45 minutes.

## References Cited in the file of this patent

## UNITED STATES PATENTS

|           |                 |               |
|-----------|-----------------|---------------|
| 2,197,357 | Widmer et al.   | Apr. 16, 1940 |
| 2,313,672 | Sälzberg et al. | Mar. 9, 1943  |
| 2,433,168 | Staeger         | Dec. 23, 1947 |
| 2,521,614 | Valyi           | Sept. 5, 1950 |
| 2,619,476 | Malinowski      | Nov. 25, 1952 |

## FOREIGN PATENTS

|         |        |               |
|---------|--------|---------------|
| 469,660 | Canada | Nov. 28, 1950 |
|---------|--------|---------------|

UNITED STATES PATENT OFFICE  
CERTIFICATE OF CORRECTION

Patent No. 2,847,388

August 12, 1958

Stuart H. Rider et al.

It is hereby certified that error appears in the printed specification of the above numbered patent requiring correction and that the said Letters Patent should read as corrected below.

Column 2, line 59, after "it" insert -- is --; column 3, line 36, for "100 parts" read 1000 parts --; lines 73 and 74, for "methyl" read -- methylol --.

Signed and sealed this 11th day of November 1958.

(SEAL)

Attest:

KARL H. AXLINE

Attesting Officer

ROBERT C. WATSON  
Commissioner of Patents